



US011719185B2

(12) **United States Patent**  
**Lineton et al.**

(10) **Patent No.:** **US 11,719,185 B2**  
(45) **Date of Patent:** **Aug. 8, 2023**

(54) **COATING TO REDUCE COKING DEPOSITS  
ON STEEL PISTONS**

(71) Applicant: **TENNECO INC.**, Lake Forest, IL (US)

(72) Inventors: **Warran Boyd Lineton**, Chelsea, MI (US); **Timothy Christopher Vezina**, Northville, MI (US)

(73) Assignee: **Tenneco Inc.**, Lake Forest, IL (US)

(\*) Notice: Subject to any disclaimer, the term of this patent is extended or adjusted under 35 U.S.C. 154(b) by 0 days.

(21) Appl. No.: **17/518,018**

(22) Filed: **Nov. 3, 2021**

(65) **Prior Publication Data**

US 2022/0065192 A1 Mar. 3, 2022

**Related U.S. Application Data**

(62) Division of application No. 15/901,783, filed on Feb. 21, 2018, now Pat. No. 11,168,643.

(51) **Int. Cl.**

**F02F 3/12** (2006.01)

**F02F 3/10** (2006.01)

**F02F 3/16** (2006.01)

(52) **U.S. Cl.**

CPC ..... **F02F 3/12** (2013.01); **F02F 3/10** (2013.01); **F02F 3/16** (2013.01); **F05C 2225/04** (2013.01); **F05C 2253/12** (2013.01)

(58) **Field of Classification Search**

CPC ..... F02F 3/12; F02F 3/10; F02F 3/16; F02F 3/0015; F02F 3/003; F02F 3/0084; F16J 1/005; F16J 1/01; F05C 2225/04; F05C 2253/12

See application file for complete search history.

(56) **References Cited**

**U.S. PATENT DOCUMENTS**

|              |   |         |          |       |             |
|--------------|---|---------|----------|-------|-------------|
| 2,817,562 A  | * | 12/1957 | Fleming  | ..... | F02F 3/10   |
|              |   |         |          |       | 92/155      |
| 5,063,894 A  | * | 11/1991 | Mielke   | ..... | C22C 23/06  |
|              |   |         |          |       | 123/193.6   |
| 5,154,109 A  | * | 10/1992 | Fluga    | ..... | F16J 1/01   |
|              |   |         |          |       | 92/248      |
| 5,490,445 A  | * | 2/1996  | Rao      | ..... | F16J 9/06   |
|              |   |         |          |       | 92/155      |
| 6,495,267 B1 | * | 12/2002 | Schenkel | ..... | C25D 11/026 |
|              |   |         |          |       | 420/407     |

(Continued)

**FOREIGN PATENT DOCUMENTS**

|    |             |        |
|----|-------------|--------|
| CN | 101784780 A | 7/2010 |
| CN | 106481478 A | 3/2017 |

(Continued)

*Primary Examiner* — Grant Moubry

(74) *Attorney, Agent, or Firm* — Robert L. Stearns; Dickinson Wright PLLC

(57) **ABSTRACT**

A piston for an internal combustion engine is provided. The piston includes a coating applied to a ferrous body portion to reduce or prevent chemical bonding of carbon deposits or coking on the body portion at temperatures ranging from 200 to 400° C. The coating includes a fluoropolymer, such as polytetrafluoroethylene, fluorosilane, fluorocarbon, fluoroplastic resin, and/or perfluoroplastic, and may be hydrocarbon or silicone based. The coating also has a thickness of 25 microns to 1 millimeter. The coating can be disposed on an undercrown surface, ring grooves, ring lands, pin bosses, and/or skirt sections of the body portion.

**8 Claims, 2 Drawing Sheets**



| (56)                     | References Cited |                            |
|--------------------------|------------------|----------------------------|
| U.S. PATENT DOCUMENTS    |                  |                            |
| 8,220,433                | B2 *             | 7/2012 Sasaki .....        |
|                          |                  | C10M 111/04<br>123/193.6   |
| 8,789,509                | B2 *             | 7/2014 Sasaki .....        |
|                          |                  | C10M 111/04<br>123/193.6   |
| 9,163,579                | B2 *             | 10/2015 Aharonov .....     |
| 9,670,870                | B2 *             | 6/2017 Bischofberger ..... |
| 9,903,310                | B2 *             | 2/2018 Bieneman .....      |
| 9,945,480                | B2 *             | 4/2018 Kantola .....       |
| 10,352,269               | B2 *             | 7/2019 Ikai .....          |
| 10,487,773               | B2 *             | 11/2019 Taguchi .....      |
| 2003/0051714             | A1 *             | 3/2003 Bedwell .....       |
|                          |                  | F02F 3/10<br>123/670       |
| 2007/0113802             | A1 *             | 5/2007 Mihara .....        |
|                          |                  | F02F 3/12<br>123/41.35     |
| 2008/0163751             | A1 *             | 7/2008 Subramanian .....   |
|                          |                  | F16J 1/01<br>29/888.048    |
| 2010/0251886             | A1 *             | 10/2010 Fussner .....      |
|                          |                  | F02F 3/105<br>92/223       |
| 2010/0294230             | A1 *             | 11/2010 Raj .....          |
|                          |                  | C10M 155/02<br>123/196 AB  |
| 2011/0139114             | A1               | 6/2011 Nakazawa et al.     |
| 2013/0133609             | A1 *             | 5/2013 Matsuo .....        |
|                          |                  | F02F 3/10<br>123/193.6     |
| 2014/0123930             | A1 *             | 5/2014 Lineton .....       |
|                          |                  | F02F 3/16<br>123/193.6     |
| 2014/0196439             | A1 *             | 7/2014 Dolan .....         |
|                          |                  | F02B 23/104<br>60/299      |
| 2015/0204233             | A1 *             | 7/2015 Nanba .....         |
|                          |                  | C23C 18/1831<br>427/302    |
| 2016/0273484             | A1 *             | 9/2016 Tateno .....        |
| 2017/0122147             | A1 *             | 5/2017 Dolan .....         |
|                          |                  | F02B 23/104                |
| 2017/0335792             | A1 *             | 11/2017 Matsuo .....       |
|                          |                  | F02F 3/0069                |
| FOREIGN PATENT DOCUMENTS |                  |                            |
| JP                       |                  | 57179354 A * 11/1982 ..... |
| JP                       |                  | F02F 3/22                  |
|                          |                  | 2014034917 A * 2/2014      |

\* cited by examiner

**FIG. 1**



FIG. 2

## 1

COATING TO REDUCE COKING DEPOSITS  
ON STEEL PISTONS

## BACKGROUND OF THE INVENTION

## 1. Field of the Invention

This invention relates generally to pistons for internal combustion engines, and methods of manufacturing the same.

## 2. Related Art

Modern heavy duty diesel engines are being pushed towards increased efficiency under emissions and fuel economy legislation. To achieve greater efficiency, the engines must run at higher temperatures. For example, some internal combustion engines are being designed to run hotter, and some types of steel pistons are designed to run at temperatures 100 to 250° C. hotter than standard pistons in some zones.

However, while desirable to increase the temperature within the combustion chamber, it remains necessary to maintain the piston at a workable temperature. As such, it is known to incorporate outer and inner cooling galleries, both open and closed, within the piston head through which engine oil is circulated to reduce the operating temperature of the piston head. The outer cooling galleries typically circulates about an upper land of the piston including a ring groove region while the inner cooling gallery is typically beneath an upper combustion surface of the piston head, commonly referred to as undercrown. Alternatively, the piston can have a galleryless design and thus has an open undercrown region for exposure to cooling oil. Both the ring belt region and the undercrown surface benefit from cooling action of the circulated oil. However, over time, the circulated oil begins to degrade and oxidize. The oxidation is driven by heating of the oil due to contact with the high temperature piston surfaces, and thus, deposits can form on the surfaces of the piston, also referred to as coking. The increased temperatures of the pistons during operation contributes to the risk of increased coking, especially in the undercrown and land regions of the piston. As the deposit build-up continues, an insulation layer is formed on the respective surfaces. Due to the coking deposits, the cooling effects of the circulated oil can be diminished, which in turn leads to combustion bowl surface oxidation and erosion, as well as over tempering of the surface. As such, the mechanical properties of the piston material are diminished, which can lead to crack formation.

## SUMMARY

One aspect of the invention provides a piston for an internal combustion engine which includes a coating for mitigating, reducing, or avoiding carbon deposits or coking during operation of the piston in the engine. The piston includes a body portion formed of a ferrous material, and the coating is disposed on the body portion. The body portion includes a crown presenting a combustion surface and an undercrown surface, and a ring belt region depending from the combustion surface. The body portion also includes a pair of pin bosses depending from the crown and spaced from one another by a pair of skirt sections. The coating includes a fluoropolymer and has a thickness of 25 microns to 1 millimeter.

## 2

Another aspect of the invention provides a method of manufacturing a piston. The method includes the steps of: providing a body portion formed of a ferrous material. The body portion includes a crown presenting a combustion surface and an undercrown surface, and a ring belt region depending from the combustion surface. The body portion also includes a pair of pin bosses depending from the crown and spaced from one another by a pair of skirt sections. The method further includes disposing a coating on the body portion. The coating includes a fluoropolymer and has a thickness of 25 microns to 1 millimeter.

## BRIEF DESCRIPTION OF THE DRAWINGS

These and other advantages of the present invention will be readily appreciated, as the same becomes better understood by reference to the following detailed description when considered in connection with the accompanying drawings wherein:

FIG. 1 is a perspective sectional view of a gallery-containing diesel engine piston including a coating applied to the crown according to an example embodiment; and

FIG. 2 is a perspective sectional view of a galleryless diesel engine piston including the coating applied to the crown according to another example embodiment.

## DETAILED DESCRIPTION OF EXEMPLARY EMBODIMENTS

One aspect of the invention provides a piston 20 with a coating 22 for use in an internal combustion engine, such as a heavy duty diesel engine or alternatively a gasoline engine. The coating 22 reduces or avoids coking deposits during operation of the piston 20 in the engine at temperatures ranging from 200 to 400° C. Thus, the piston 20 can provide for improved cooling effects of the circulated oil, which in turn leads to reduced surface oxidation and erosion, as well as reduced tempering of the surface. As such, the mechanical properties of the piston 20 are improved, and crack formation is reduced. Examples of the piston 20 are shown in FIGS. 1 and 2. However, the coating 22 can be applied to pistons having other designs.

According to the example embodiments of FIGS. 1 and 2, the piston 20 includes a body portion 24 formed of a ferrous material, such as steel or another iron-based material. The body portion 24 extends around a center axis A and longitudinally along the center axis A from an upper end 26 to a lower end 28. The body portion 24 includes a crown 30 presenting a combustion surface 32 at the upper end 26 for exposure to a combustion chamber of the internal combustion engine. The combustion surface 32 includes a combustion bowl extending toward the center axis A from an outer rim and includes an apex at the center axis A. The crown 30 also includes an undercrown surface 34 located opposite the combustion surface 32 which is typically exposed to cooling oil or another cooling medium.

The body portion 24 further includes a ring belt region 36 depending from the combustion surface 32. The ring belt region 36 includes a plurality of ring grooves 36a spaced from one another by lands 36b. The ring belt region 36 is located at an outer diameter of the body portion 24 and extends circumferentially about the center axis A of the body portion 24.

The body portion 24 further includes a pair of pin bosses 38 depending from the crown 30 and spaced from one another by a pair of skirt sections 40. The pin bosses 38 and

the skirt sections 40 extend from the crown 30 to the lower end 28, and the pin bosses 38 define a pin bore for receiving a wrist pin (not shown).

According to the example embodiment of FIG. 1, the body portion 24 of the piston 20 includes a closed or sealed cooling gallery 42 extending circumferentially around the center axis A between the crown 30 and a lower section of the body portion 24. The lower section of the body portion 24 includes at least a portion of the ring belt region 36, the pin bosses 38, and the skirt sections 40. In this embodiment, the crown 30 includes an upper rib 44 spaced from the center axis A and extending circumferentially around the center axis A. The lower section of the body portion 24 includes a lower rib 46 aligned with the upper rib 44 and extending circumferentially around the center axis A. The upper rib 44 and the lower rib 46 are joined, typically by welding, for example friction welding and/or laser welding. The lower section of the body portion 24 also includes a lower wall 48 extending radially from the lower rib, 46 to the ring belt region 36. As shown in FIG. 1, the cooling gallery 42 extends circumferentially around the center axis A of the body portion 24 and defined by the ring belt region 36, the ribs, the undercrown surface 34, and the lower wall 48.

According to the example embodiment of FIG. 2, the body portion 24 of the piston 20 is galleryless. Thus, the undercrown surface 34 is openly exposed and not bounded by a sealed or enclosed cooling gallery 42. The undercrown surface 34 is located both opposite the combustion surface 32 and radially inwardly of the ring grooves 36a. The undercrown surface 34 includes a center region disposed at the center axis A and between the pin bosses 38 and the skirt sections 40, which is open for exposure to cooling oil. The undercrown surface 34 also includes pockets 50 disposed between the pin bosses 38 and the ring belt region 36, which are also open for exposure to cooling oil.

The coating 22 of the piston 20 is disposed on at least a portion of the ferrous body portion 24. For example, the coating 22 is disposed on at least one of the undercrown surface 34, at least one of the ring grooves 36a, at least one of the lands 36b, at least one of the pin bosses 38, and at least one of the skirt sections 40. In the example embodiments of FIGS. 1 and 2, the coating 22 is disposed on an uppermost land 36b of the crown 30. However, the coating 22 could be located on another other section of the body portion 24. The coating 22 is applied when the piston 20 is otherwise in the finished condition.

As stated above, the coating 22 reduces or avoids the bonding of the carbon deposits on the body portion 24 of the piston 20, also referred to as coking, during operation of the piston 20 in the engine at service temperatures ranging from 200 to 400° C. The coating 22 includes a fluoropolymer and has a thickness of 25 microns to 1 millimeter. The thickness of the coating 22 is measured after the coating 22 is dried and cured. For example, the fluoropolymer of the coating 22 can include polytetrafluoroethylene (PTFE), fluorosilane, fluorocarbon, fluoroplastic resin, and/or perfluoroplastic. According to one embodiment, the coating 22 further includes silicone, polysilane, and/or polysilazane, and the coating 22 may be silicone-based. The coating 22 could alternatively be another non-stick formulation which includes a fluoropolymer. For example, the coating 22 could be hydrocarbon based. In another embodiment the coating 22 includes a thermoset binder. For example, the thermoset can include phenolic, epoxy, polyester, polyamide-imide or any combination of the thermoset resins. The fluoropolymer is added to the uncured thermoset resin(s) and mixed before application to one or more surfaces of the piston 20 followed

by curing. Alternatively, the fluoro-polymer can be added to the thermoplastic resin as uncured components and copolymerized in the curing step of the coating 22. In both methods, the fluoropolymer components segregate to the surface of the coating 22 over time and provide the non-stick effect.

Another aspect of the invention provides a method of manufacturing the piston 20. The method includes providing the body portion 24 formed of a ferrous material. The body portion 24 can include the design described above, or can have a different design.

The method further includes disposing the coating 22 on the body portion 24. The coating 22 includes the fluoropolymer as described above. The step of disposing the coating 22 on the body portion 24 includes disposing the coating 22 on at least one of the following: the undercrown surface 34, at least one ring groove 36a of the ring belt region 36, at least one land 36b of the ring belt region 36, at least one of the pin bosses 38, and at least one of the skirt sections 40. The coating 22 is preferably applied by spraying, dipping, brushing, ink-jet, rolling, pipetting or transfer stamping.

The coating step is preferably a rapid and atmospheric method. According to an example embodiment, the spraying step is conducted using an airbrush dispenser. The spraying should be capable of directing the coating 22 to specific regions of the body portion 24. The method can also include masking a portion or portions of the body portion 24, to prevent the coating 22 from being applied to that portion or portions, during the spraying step. The method can also include moving the body portion 24 relative to the airbrush dispenser during the spraying step. When manufacturing multiple pistons 20, a part handling and manipulation system can be used to pick and place the body portions 24 and move them appropriately in a spray jet. Alternatively a system of linear axis slides or a robot could manipulate the spray gun relative to the body portion 24. The method next includes drying and curing the coating 22. A convection oven or infrared lamps can be used to dry and/or cure the coating 22. The thickness of the coating 22 is 25 microns to 1 millimeter after the drying and curing steps.

The method of manufacturing the coated piston 20 has no need for vacuum chambers or special atmospheres that would be needed in physical vapor deposition or chemical vapor deposition. Thus, the process of manufacturing the coated piston 20 is a production friendly, minimally invasive process. It can fit with current production methods, and the coating 22 could be applied over the top of a finished phosphated piston. Initial testing conducted in an engine run at full power for 25 hours showed coking deposits on the undercrown of non-coated, standard pistons, but the coated piston 20 run in the same test had the coking deposits significantly reduced (by 66%).

Obviously, many modifications and variations of the present invention are possible in light of the above teachings and may be practiced otherwise than as specifically described while within the scope of the following claims. In particular, all features of all claims and of all embodiments can be combined with each other, as long as they do not contradict each other.

The invention claimed is:

1. A method of manufacturing a piston, comprising the steps of:  
providing a body portion formed of a ferrous material, the body portion including a crown presenting a combustion surface and an undercrown surface, the body portion including a ring belt region depending from the combustion surface, the body portion including a pair

of pin bosses depending from the crown and spaced from one another by a pair of skirt sections, and disposing a coating on the body portion, the coating including a fluoropolymer and having a thickness of 25 microns to 1 millimeter, wherein the coating is disposed on the body portion by spraying, dipping, brushing, ink-jet, rolling, pipetting, or transfer stamping the coating on the body portion, and curing the coated body portion.

2. The method of claim 1, wherein the coating further includes silicone, polysilane, polysilazane, and/or a thermoset resin.

3. The method of claim 1, wherein the fluoropolymer of the coating includes polytetrafluoroethylene, fluorosilane, fluorocarbon, fluoroplastic resin, and/or perfluoroplastic.

4. The method of claim 1, wherein the coating reduces chemical bonding of carbon deposits or coking on the body portion at temperatures ranging from 200 to 400° C.

5. The method of claim 1, wherein the step of disposing the coating on the body portion includes disposing the coating on at least one of the following: the undercrown surface, at least one ring groove of the ring belt region, at least one land of the ring belt region, at least one of the pin bosses, and at least one of the skirt sections.

6. The method of claim 1, wherein the coating is disposed on the body portion by spraying, and the spraying step is conducted using an airbrush dispenser.

7. The method of claim 1, wherein the curing step is conducted in a convection oven or by infrared lamps.

8. The method of claim 1, wherein the coating is disposed on the body portion by spraying, and further including masking a portion of the body portion during spraying, and moving the body portion relative to an airbrush dispenser during spraying.

\* \* \* \* \*